

## UNITED STATES PATENT OFFICE

JOHANN WEISS, OF VIENNA, AUSTRIA

## LIGHT METAL ALLOY

No Drawing. Application filed May 25, 1929, Serial No. 366,088, and in France November 23, 1928.

The light metal alloys hitherto used for the pistons of internal combustion engines are for the most part aluminum-copper-alloys with addition of silicon, iron, manganese and the like. But, the addition of silicon or manganese has the drawback that the alloys become comparatively hard, the cylinder-walls thereby and on account of the small sliding power being worn out within a 10 comparatively short time. The hardness of the alloy impairs also its capability of being worked. Furthermore it is difficult to avoid porosity of the casting.

According to the present invention the alloy consists of aluminum, of 12 to 18 parts by weight of copper, of 0.1 to 5 parts of magnesium and of 0.1 to 5 parts of nickel, sum total 100 parts by weight.

Also nearly 0.05 to 8 parts by weight of 20 iron or the like may be added to the said alloy.

The alloy according to the invention allows to produce without trouble a homogeneous and dense casting; the material is easily workable; the heat conductivity is very high; the pistons made of such a material have a high sliding power. According to the proportions employed the specific weight is 2.9 to 3.1, the ball test hardness is 140 to 30 150 and the strength is 20 to 22 kg/mm<sup>2</sup>.

Of course, this alloy may also be used for other objects than pistons, especially for the connecting-rod of internal combustion engines or for other parts of machines.

What I claim is:

1. A light metal alloy consisting of: aluminum, 12 to 18 parts by weight of copper 0.1 to 5.00 parts by weight of magnesium, 0.1 to 5 parts by weight of nickel, the total sum 40 being 100 parts by weight.

2. A light metal alloy consisting of: aluminum, 12 to 18 parts by weight of copper 0.1 to 5.00 parts by weight of magnesium, 0.1 to 5 parts by weight of nickel and of 0.05 to 8 45 parts by weight of iron, the total sum being 100 parts by weight.

Signed at Vienna, Austria, this 11th day of May, 1929.

JOHANN WEISS.